

W. D. WOOD.  
ANNEALING SHEET IRON.

No. 66,546.

Patented July 9, 1867.



Witnesses:

W. D. Lewis

Allan C. Bakewell

Inventor:

W. D. George Wood

by his atty

Bakewell & Crisby

# United States Patent Office.

W. DEWEES WOOD, OF THE BOROUGH OF MCKEESPORT, PENNSYLVANIA.

Letters Patent No. 66,546, dated July 9, 1867.

## IMPROVEMENT IN ANNEALING SHEET IRON.

The Schedule referred to in these Letters Patent and making part of the same.

TO ALL WHOM IT MAY CONCERN:

Be it known that I, W. DEWEES WOOD, of the borough of McKeesport, in the county of Allegheny, and State of Pennsylvania, have invented a new and useful Improvement in the Process of Annealing Sheet-Iron; and I do hereby declare the following to be a full, clear, and exact description thereof, reference being had to the accompanying drawing, forming part of this specification, in which—

Figure 1 is a perspective representation of my improved annealing-box.

Figure 2 is a transverse vertical section.

In both figures like letters of reference denote similar parts.

Sheets of iron and other metals are annealed by placing them in piles within a heavy cast-iron box, from which the external air is excluded by closing the joints with sand, and placing the box with its contents in a furnace, in which it is exposed to a high heat, and then afterwards gradually cooled. These cast-iron annealing-boxes are necessarily made very heavy, in order that they may preserve their shape when exposed to the heat of the annealing furnace, because, when they become warped and misshapen, they are useless, as it is then impossible to close them so as to exclude the air. They are usually made to weigh about four tons, and are very expensive, but notwithstanding their heaviness, they last only a short time before they become so twisted and warped as to be no longer fit for use. Another practical difficulty in the use of annealing-boxes for sheet iron is that the sheets of metal become discolored at their edges, the discoloration being owing to the effect of the air which surrounds the pile of sheets in the box, and which is contained in the box when it is closed up. These difficulties, viz., the warping of the annealing-box and the discoloration of the sheets during the annealing process, I propose to remedy in a great degree by my improvement, which consists in compressing together the sheets of iron or other metal within the annealing-box between the parallel surfaces of its bottom and cover, and screwing, or otherwise forcibly holding, together, the top and bottom pieces of the box, so as not only to prevent the warping of the box, but also prevent the entrance of air between the layers.

To enable others skilled in the art to construct and use my improved annealing-box, I will proceed to describe its construction and the manner in which it is to be used.

In the accompanying drawing *a* is the bottom piece or bed-plate of the annealing-box, consisting of a plate of cast iron, rectangular in shape, with a plane surface on the upper side and a raised ledge or rim *b* around its edge, on all four sides, for the purpose of retaining the sand packed around the box to exclude the air. The under side of the bed-plate *a* is furnished with boxes *c* for the reception of flanged truck-wheels *d*, so placed that the box may be run in and out of the annealing-furnace on a rail track, *e e*. The upper piece or box *f* consists of four sides and a top, cast in one piece. It is strengthened by a rib, *g*, extending along each side from end to end, and the top of the box extends beyond the sides all round, so as to form a ledge, *h*, projecting as far as the outer edge of the bottom piece *a*. The upper piece *f* thus forms a box having a rectangular cavity, which is placed with the open bottom downwards on the bottom piece or bed-plate *a*, as shown in fig. 2, the sides of the box being inside the raised rim *b*, and not quite touching it, so as to allow sand to be packed between the rim *b* and the sides of the box *f*. The box piece *f* is fastened to the bed-plate *a* by means of clamps *k* placed at suitable intervals on each side and at both ends. The clamps *k* have a T head, *i*, at one end, and a tapering recess or mortise near the other end, to receive a wedge-shaped key, *n*. These clamps are placed vertically on the sides of the box, and are let into suitable recesses *m m'* in the rim of the bed-plate *a* and in the ledge of the box piece *f*, the T head resting against the under side of the rim of the bed-plate *a*. Near each of the four corners of the box, in the ledge *h* of the box, is a round hole, *x*, to receive the end of a screw-bolt, *p*, which has a T head at the other end, the bolt entering a recess, *q*, in the rim of the bed-plate, and the T head resting against the under side of the rim of the bed-plate. The upper end of these bolts *p* is chased with screw-threads, and a nut, *r*, screwed on the bolt, serves to force down the box *f* on the bed-plate *a*, and press together the sheets of iron placed in the box between its cover and the bed-plate *a*.

The mode of using my improved annealing-box is as follows: The box piece *f*, being hoisted by a crane or otherwise from the bed-plate *a*, the sheets of metal to be annealed are placed one on top of another in layers on the bed-plate, forming a pile so high that when compressed the bottom of the box piece *f* shall not quite touch the surface of the bed-plate *a*. The box is then placed over the pile of sheets, and the screw-bolts *p* are

inserted at the four corners of the box, and the nuts *r* screwed down until the sheets are compactly pressed together. If preferred, this may be done by an hydraulic or other press instead of by screw-bolts. While the box *f* is thus pressed down on to the sheets of metal, the clamps *k* are inserted into their respective grooves or recesses, and the keys *n* are driven into their mortises, so as to hold the box *f* firmly down to its place. The screw-bolts *p* are then removed, as the heat of the annealing furnace would injure them, and the box is ready to be run into the furnace. The mode of fastening together the box and bed-plate, which I have described, I consider most convenient, although others may be used, such as clamps surrounding or partially surrounding the box. When thus rigidly connected together and allowed to cool before the clamps are removed, the box piece and bed-plate retain their shape, and can be used repeatedly for a long time. The effect produced by thus rigidly compressing together the sheets of iron during the process of annealing is greatly to improve their appearance and finish. This is especially important in the manufacture of glazed or polished sheet iron, (known as imitation Russia,) where so much depends on uniformity of color. In the ordinary mode of annealing, although the sheets are pressed down merely by the weight of the annealing-box, yet the air within the box finds its way between the layers of metal, and produces considerable discoloration; but by my method of rigidly compressing the sheets together they are brought so closely in contact with each other that the air can only penetrate a very slight distance at the edges, so that the sheets are of uniform color and finish, excepting just at their margin. This compression of the sheets, as distinguished from mere pressure by superimposed weight, may be also obtained by placing them between plates screwed together to form a solid pack, which is placed in an annealing-box; but this is not so desirable, as it leaves mere air space around the iron in the box, and the screw-together of the box, as before described, accomplishes the desired result, whilst it also preserves the box from warping.

What I claim as my invention, and desire to secure by Letters Patent, is—

1. The use, in the process of annealing sheet iron, of boxes so constructed, substantially as hereinbefore described, as that the sheets may be compressed between the top and bottom of the box, for the purpose of preventing their discoloration.
2. The use of annealing-boxes, so constructed as that the box piece and bottom piece may be clamped or securely fastened together, for the purpose of preserving the shape of the box and preventing its warping while cooling, substantially as hereinbefore described.
3. Annealing imitation Russia or other glazed or polished sheet iron, in packs or layers, forcibly compressed together, and held under rigid compression during the process of annealing.

In testimony whereof I, the said W. DEWEES WOOD, have hereunto set my hand in presence of—

W. DEWEES WOOD.

Witnesses:

ALLAN C. BAKEWELL,  
W. BAKEWELL.